



US008074750B2

(12) **United States Patent**  
**Choe et al.**

(10) **Patent No.:** **US 8,074,750 B2**  
(b5) **Date of Patent:** **Dec. 13, 2011**

(54) **EARTH-BORING TOOLS COMPRISING SILICON CARBIDE COMPOSITE MATERIALS, AND METHODS OF FORMING SAME**

(75) Inventors: **Heeman Choe**, Seoul (KR); **John H. Stevens**, Spring, TX (US); **James L. Overstreet**, Tomball, TX (US); **Jimmy W. Eason**, The Woodlands, TX (US); **James C. Westhoff**, The Woodlands, TX (US)

(73) Assignee: **Baker Hughes Incorporated**, Houston, TX (US)

(\*) Notice: Subject to any disclaimer, the term of this patent is extended or adjusted under 35 U.S.C. 154(b) by 0 days.

(21) Appl. No.: **12/875,570**

(22) Filed: **Sep. 3, 2010**

(65) **Prior Publication Data**

US 2010/0326739 A1 Dec. 30, 2010

**Related U.S. Application Data**

(60) Division of application No. 11/965,018, filed on Dec. 27, 2007, now Pat. No. 7,807,099, which is a continuation-in-part of application No. 11/271,153, filed on Nov. 10, 2005, now Pat. No. 7,802,495, and a continuation-in-part of application No. 11/272,439, filed on Nov. 10, 2005, now Pat. No. 7,776,256.

(51) **Int. Cl.**

**E21B 10/00** (2006.01)  
**B22D 19/14** (2006.01)

(52) **U.S. Cl.** ..... **175/425**; 175/374; 75/236; 75/249; 164/97; 164/98

(58) **Field of Classification Search** ..... 75/249, 75/236; 419/14; 175/374, 425; 164/97, 164/98

See application file for complete search history.

(56) **References Cited**

U.S. PATENT DOCUMENTS

|             |         |                 |
|-------------|---------|-----------------|
| 1,676,887 A | 7/1928  | Chamberlin      |
| 1,954,166 A | 4/1934  | Campbell        |
| 2,299,207 A | 10/1942 | Bevillard       |
| 2,507,439 A | 5/1950  | Goolsbee        |
| 2,819,958 A | 1/1958  | Abkowitz et al. |
| 2,819,959 A | 1/1958  | Abkowitz        |
| 2,906,654 A | 9/1959  | Abkowitz        |
| 3,368,881 A | 2/1968  | Abkowitz et al. |
| 3,471,921 A | 10/1969 | Feeenstra       |
| 3,660,050 A | 5/1972  | Iler et al.     |
| 3,757,878 A | 9/1973  | Wilder et al.   |
| 3,757,879 A | 9/1973  | Wilder et al.   |
| 3,841,852 A | 10/1974 | Wilder et al.   |
| 3,880,971 A | 4/1975  | Pantanelli      |
| 3,987,859 A | 10/1976 | Lichte          |
| 4,017,480 A | 4/1977  | Baum            |
| 4,047,828 A | 9/1977  | Makely          |
| 4,094,709 A | 6/1978  | Rozmus          |
| 4,098,363 A | 7/1978  | Rohde et al.    |

|             |         |                  |
|-------------|---------|------------------|
| 4,128,136 A | 12/1978 | Generoux         |
| 4,134,759 A | 1/1979  | Yajima et al.    |
| 4,157,122 A | 6/1979  | Morris           |
| 4,198,233 A | 4/1980  | Frehn            |
| 4,221,270 A | 9/1980  | Vezirian         |
| 4,229,638 A | 10/1980 | Lichte           |
| 4,233,720 A | 11/1980 | Rozmus           |
| 4,252,202 A | 2/1981  | Purser, Sr.      |
| 4,255,165 A | 3/1981  | Dennis et al.    |
| 4,306,139 A | 12/1981 | Shinozaki et al. |
| 4,341,557 A | 7/1982  | Lizenby          |
| 4,389,952 A | 6/1983  | Dreier et al.    |
| 4,398,952 A | 8/1983  | Drake            |
| 4,453,605 A | 6/1984  | Short et al.     |
| 4,499,048 A | 2/1985  | Hanejko          |
| 4,499,795 A | 2/1985  | Radtke           |
| 4,499,958 A | 2/1985  | Radtke et al.    |
| 4,503,009 A | 3/1985  | Asaka            |
| 4,526,748 A | 7/1985  | Rozmus           |
| 4,552,232 A | 11/1985 | Frear            |
| 4,554,130 A | 11/1985 | Ecer             |
| 4,562,990 A | 1/1986  | Rose             |
| 4,596,694 A | 6/1986  | Rozmus           |
| 4,597,730 A | 7/1986  | Rozmus           |
| 4,620,600 A | 11/1986 | Persson          |

(Continued)

FOREIGN PATENT DOCUMENTS

AU 695583 2/1998

(Continued)

OTHER PUBLICATIONS

"Boron Carbide Nozzles and Inserts," Seven Stars International webpage <http://www.concentric.net/~ctkang/nozzle.shtml>, printed Sep. 7, 2006, 8 pages.

"Heat Treating of Titanium and Titanium Alloys," Key to Metals website article, [www.key-to-metals.com](http://www.key-to-metals.com), printed Sep. 21, 2006, 7 pages.

Al-Haidary, J.T., et al., "Evaluation Study of Cast Al-SiCp Composites," Materials Science-Poland, vol. 25, No. 1, 2007.

Alman et al., "The Abrasive Wear of Sintered Titanium Matrix-Ceramic Particle Reinforced Composites," WEAR, 225-229, pp. 629-639, 1999.

(Continued)

*Primary Examiner* — Roy King

*Assistant Examiner* — Ngoclan Mai

(74) *Attorney, Agent, or Firm* — TraskBritt

(57) **ABSTRACT**

Earth-boring tools for drilling subterranean formations include a particle-matrix composite material comprising a plurality of silicon carbide particles dispersed throughout a matrix material, such as, for example, an aluminum or aluminum-based alloy. In some embodiments, the silicon carbide particles comprise an ABC-SiC material. Methods of manufacturing such tools include providing a plurality of silicon carbide particles within a matrix material. Optionally, the silicon carbide particles may comprise ABC-SiC material, and the ABC-SiC material may be toughened to increase a fracture toughness exhibited by the ABC-SiC material. In some methods, at least one of an infiltration process and a powder compaction and consolidation process may be employed.

## U.S. PATENT DOCUMENTS

|               |         |                    |                 |         |                    |
|---------------|---------|--------------------|-----------------|---------|--------------------|
| 4,686,080 A   | 8/1987  | Hara et al.        | 5,856,626 A     | 1/1999  | Fischer et al.     |
| 4,694,919 A   | 9/1987  | Barr               | 5,865,571 A     | 2/1999  | Tankala et al.     |
| 4,738,322 A   | 4/1988  | Hall et al.        | 5,878,634 A     | 3/1999  | Tibbitts           |
| 4,743,515 A   | 5/1988  | Fischer et al.     | 5,880,382 A     | 3/1999  | Fang et al.        |
| 4,744,943 A   | 5/1988  | Timm               | 5,897,830 A     | 4/1999  | Abkowitz et al.    |
| 4,774,211 A   | 9/1988  | Hamilton et al.    | 5,904,212 A     | 5/1999  | Arfele             |
| 4,809,903 A   | 3/1989  | Eylon et al.       | 5,947,214 A     | 9/1999  | Tibbitts           |
| 4,838,366 A   | 6/1989  | Jones              | 5,957,006 A     | 9/1999  | Smith              |
| 4,871,377 A   | 10/1989 | Frushour           | 5,963,775 A     | 10/1999 | Fang               |
| 4,881,431 A   | 11/1989 | Bieneck            | 5,967,248 A     | 10/1999 | Drake et al.       |
| 4,884,477 A   | 12/1989 | Smith et al.       | 5,979,575 A     | 11/1999 | Overstreet et al.  |
| 4,889,017 A   | 12/1989 | Fuller et al.      | 5,980,602 A     | 11/1999 | Carden             |
| 4,919,013 A   | 4/1990  | Smith et al.       | 6,029,544 A     | 2/2000  | Katayama           |
| 4,923,512 A   | 5/1990  | Timm et al.        | 6,045,750 A     | 4/2000  | Drake et al.       |
| 4,940,099 A   | 7/1990  | Deane et al.       | 6,051,171 A     | 4/2000  | Takeuchi et al.    |
| 4,956,012 A   | 9/1990  | Jacobs et al.      | 6,063,333 A     | 5/2000  | Dennis             |
| 4,968,348 A   | 11/1990 | Abkowitz et al.    | 6,068,070 A     | 5/2000  | Scott              |
| 4,981,665 A   | 1/1991  | Boecker et al.     | 6,073,518 A     | 6/2000  | Chow et al.        |
| 5,000,273 A   | 3/1991  | Horton et al.      | 6,086,980 A     | 7/2000  | Foster et al.      |
| 5,030,598 A   | 7/1991  | Hsieh              | 6,089,123 A     | 7/2000  | Chow et al.        |
| 5,032,352 A   | 7/1991  | Meeks et al.       | 6,099,664 A     | 8/2000  | Davies et al.      |
| 5,049,450 A   | 9/1991  | Dorfman et al.     | 6,148,936 A     | 11/2000 | Evans et al.       |
| 5,090,491 A   | 2/1992  | Tibbitts et al.    | 6,200,514 B1    | 3/2001  | Meister            |
| 5,101,692 A   | 4/1992  | Simpson            | 6,209,420 B1    | 4/2001  | Butcher et al.     |
| 5,150,636 A   | 9/1992  | Hill               | 6,214,134 B1    | 4/2001  | Eylon et al.       |
| 5,161,898 A   | 11/1992 | Drake              | 6,214,287 B1    | 4/2001  | Waldenstrom        |
| 5,232,522 A   | 8/1993  | Doktycz et al.     | 6,220,117 B1    | 4/2001  | Butcher            |
| 5,281,260 A   | 1/1994  | Kumar et al.       | 6,227,188 B1    | 5/2001  | Tankala et al.     |
| 5,286,685 A   | 2/1994  | Schoennahl et al.  | 6,228,139 B1    | 5/2001  | Oskarrson          |
| 5,311,958 A   | 5/1994  | Isbell et al.      | 6,241,036 B1    | 6/2001  | Lovato et al.      |
| 5,322,139 A   | 6/1994  | Rose et al.        | 6,254,658 B1    | 7/2001  | Taniuchi et al.    |
| 5,333,699 A   | 8/1994  | Thigpen et al.     | 6,284,014 B1    | 9/2001  | Carden             |
| 5,348,806 A   | 9/1994  | Kojo et al.        | 6,287,360 B1    | 9/2001  | Kembaiyan et al.   |
| 5,372,777 A * | 12/1994 | Yang .....         | 6,290,438 B1    | 9/2001  | Papajewski         |
| 5,373,907 A   | 12/1994 | Weaver             | 6,293,986 B1    | 9/2001  | Rodiger et al.     |
| 5,433,280 A   | 7/1995  | Smith              | 6,322,746 B1    | 11/2001 | LaSalle et al.     |
| 5,439,068 A   | 8/1995  | Huffstutter et al. | 6,348,110 B1    | 2/2002  | Evans              |
| 5,443,337 A   | 8/1995  | Katayama           | 6,375,706 B2    | 4/2002  | Kembaiyan et al.   |
| 5,445,231 A   | 8/1995  | Scott et al.       | 6,408,958 B1    | 6/2002  | Isbell et al.      |
| 5,455,000 A   | 10/1995 | Seyferth et al.    | 6,453,899 B1    | 9/2002  | Tselesin           |
| 5,467,669 A   | 11/1995 | stroud             | 6,454,025 B1    | 9/2002  | Runquist et al.    |
| 5,479,997 A   | 1/1996  | Scott et al.       | 6,454,028 B1    | 9/2002  | Evans              |
| 5,482,670 A   | 1/1996  | Hong               | 6,454,030 B1    | 9/2002  | Findley et al.     |
| 5,484,468 A   | 1/1996  | Ostlund et al.     | 6,458,471 B2    | 10/2002 | Lovato et al.      |
| 5,492,186 A   | 2/1996  | Overstreet et al.  | 6,474,425 B1    | 11/2002 | Truax et al.       |
| 5,506,055 A   | 4/1996  | Dorfman et al.     | 6,500,226 B1    | 12/2002 | Dennis             |
| 5,541,006 A   | 7/1996  | Conley             | 6,503,572 B1    | 1/2003  | Waggoner et al.    |
| 5,543,235 A   | 8/1996  | Mirchandani et al. | 6,511,265 B1    | 1/2003  | Mirchandani et al. |
| 5,544,550 A   | 8/1996  | Smith              | 6,576,182 B1    | 6/2003  | Ravagni et al.     |
| 5,560,440 A   | 10/1996 | Tibbitts           | 6,589,640 B2    | 7/2003  | Griffin et al.     |
| 5,586,612 A   | 12/1996 | Isbell et al.      | 6,607,693 B1    | 8/2003  | Saito et al.       |
| 5,593,474 A   | 1/1997  | Keshavan et al.    | 6,615,935 B2    | 9/2003  | Fang et al.        |
| 5,611,251 A   | 3/1997  | Katayama           | 6,655,481 B2    | 12/2003 | Findley et al.     |
| 5,612,264 A   | 3/1997  | Nilsson et al.     | 6,685,880 B2    | 2/2004  | Engstrom et al.    |
| 5,624,002 A   | 4/1997  | Huffstutter        | 6,742,608 B2    | 6/2004  | Murdoch            |
| 5,641,251 A   | 6/1997  | Leins et al.       | 6,742,611 B1    | 6/2004  | Illerhaus et al.   |
| 5,641,921 A   | 6/1997  | Dennis et al.      | 6,756,009 B2    | 6/2004  | Sim et al.         |
| 5,662,183 A   | 9/1997  | Fang               | 6,766,870 B2    | 7/2004  | Overstreet         |
| 5,666,864 A   | 9/1997  | Tibbitts           | 6,782,958 B2    | 8/2004  | Liang et al.       |
| 5,677,042 A   | 10/1997 | Massa et al.       | 6,849,231 B2    | 2/2005  | Kojima et al.      |
| 5,679,445 A   | 10/1997 | Massa et al.       | 6,862,970 B2    | 3/2005  | Aghajanian et al.  |
| 5,697,046 A   | 12/1997 | Conley             | 6,908,688 B1    | 6/2005  | Majagi et al.      |
| 5,697,462 A   | 12/1997 | Grimes et al.      | 6,918,942 B2    | 7/2005  | Hatta et al.       |
| 5,710,969 A   | 1/1998  | Newman             | 6,995,103 B2    | 2/2006  | Aghajanian         |
| 5,725,827 A   | 3/1998  | Rhodes et al.      | 7,044,243 B2    | 5/2006  | Kembaiyan et al.   |
| 5,732,783 A   | 3/1998  | Truax et al.       | 7,048,081 B2    | 5/2006  | Smith et al.       |
| 5,733,649 A   | 3/1998  | Kelley et al.      | 7,395,882 B2    | 7/2008  | Oldham et al.      |
| 5,733,664 A   | 3/1998  | Kelley et al.      | 7,513,320 B2    | 4/2009  | Mirchandani et al. |
| 5,740,872 A   | 4/1998  | Smith              | 2002/004105 A1  | 1/2002  | Kunze et al.       |
| 5,753,160 A   | 5/1998  | Takeuchi et al.    | 2003/0010409 A1 | 1/2003  | Kunze et al.       |
| 5,765,095 A   | 6/1998  | Flak et al.        | 2004/007393 A1  | 1/2004  | Griffin            |
| 5,776,593 A   | 7/1998  | Massa et al.       | 2004/0013558 A1 | 1/2004  | Kondoh et al.      |
| 5,778,301 A   | 7/1998  | Hong               | 2004/0060742 A1 | 4/2004  | Kembaiyan et al.   |
| 5,789,686 A   | 8/1998  | Massa et al.       | 2004/0196638 A1 | 10/2004 | Lee et al.         |
| 5,792,403 A   | 8/1998  | Massa et al.       | 2004/0243241 A1 | 12/2004 | Istephanous et al. |
| 5,806,934 A   | 9/1998  | Massa et al.       | 2004/0245022 A1 | 12/2004 | Izaguirre et al.   |
| 5,829,539 A   | 11/1998 | Newton et al.      | 2004/0245024 A1 | 12/2004 | Kembaiyan          |
| 5,830,256 A   | 11/1998 | Northrop et al.    | 2005/0008524 A1 | 1/2005  | Testani            |
|               |         |                    | 2005/0072496 A1 | 4/2005  | Hwang et al.       |

|                 |         |                    |                                                                                                                                                                                                                                                     |
|-----------------|---------|--------------------|-----------------------------------------------------------------------------------------------------------------------------------------------------------------------------------------------------------------------------------------------------|
| 2005/0084407 A1 | 4/2005  | Myrick             | International Search Report and Written Opinion of the International Search Authority for International Application No. PCT/US2006/043669, mailed Apr. 13, 2007.                                                                                    |
| 2005/0117984 A1 | 6/2005  | Eason et al.       | International Search Report and Written Opinion of the International Search Authority for International Application No. PCT/US2006/043670, mailed Apr. 2, 2007.                                                                                     |
| 2005/0126334 A1 | 6/2005  | Mirchandani        | International Search Report for International Application No. PCT/US2009/046812 dated Jan. 26, 2010, 5 pages.                                                                                                                                       |
| 2005/0211474 A1 | 9/2005  | Nguyen et al.      | International Search Report for International Application No. PCT/US2007/023275, mailed Apr. 11, 2008.                                                                                                                                              |
| 2005/0211475 A1 | 9/2005  | Mirchandani et al. | International Written Opinion for International Application No. PCT/US2009/046812 dated Jan. 26, 2010, 5 pages.                                                                                                                                     |
| 2005/0247491 A1 | 11/2005 | Mirchandani et al. | Key-To-Nonferrous, "Aluminum Matrix Composites with Discontinuous Silicon Carbide Reinforcement," <a href="http://www.key-to-nonferrous.com">http://www.key-to-nonferrous.com</a> , 3 pages, downloaded Aug. 27, 2007.                              |
| 2005/0268746 A1 | 12/2005 | Abkowitz et al.    | M Cubed Technologies Inc., "Cast Silicon Carbide Particulate-Reinforced Aluminum (Al/SiC) Metal Matrix Composites," Technote, Cast MMC, Rev. 02, 3 pages, May 8, 2001.                                                                              |
| 2006/0016521 A1 | 1/2006  | Hanusiaik et al.   | Mabuchi, M., et al., "Very High Strain-Rate Superplasticity in a Particulate Si <sub>3</sub> N <sub>4</sub> /6061 Aluminum Composite," Scripta Metallurgica et Materialia, vol. 25, No. 11, pp. 2517-2520, Copyright (c) Pergamon Press plc., 1991. |
| 2006/0032677 A1 | 2/2006  | Azar et al.        | Miserez et al. "Particle Reinforced Metals of High Ceramic Content," Material Science and Engineering A 387-389, pp. 822-831, Elsevier., 2004.                                                                                                      |
| 2006/0043648 A1 | 3/2006  | Takeuchi et al.    | Moberlychan, W.J., et al., "Controlling Interface Chemistry and Structure to Process and Toughen Silicon Carbide," Acta mater., vol. 46, No. 7, pp. 2471-2477, 1998.                                                                                |
| 2006/0057017 A1 | 3/2006  | Woodfield et al.   | Moberlychan, W.J., et al., "The Roles of Amorphous Grain Boundaries and the $\beta$ - $\alpha$ Transformation in Toughening SiC," Acta mater., vol. 46, No. 5, pp. 1625-1635, 1998.                                                                 |
| 2006/0131081 A1 | 6/2006  | Mirchandani et al. | PCT International Search Report for International Application No. PCT/US2008/087647, mailed Jul. 23, 2009, 5 pages.                                                                                                                                 |
| 2006/0231293 A1 | 10/2006 | Ladi et al.        | PCT International Written Opinion for International Application No. PCT/US2008/087647, mailed Jul. 23, 2009, 5 pages.                                                                                                                               |
| 2007/0042217 A1 | 2/2007  | Fang et al.        | Pruthviraj, R.D., et al., "Friction and Wear of Al6061 Containing 10wt.% SiC Metal Matrix Composites," International Journal of Material Science, vol. 2, No. 1, pp. 59-64, 2007.                                                                   |
| 2007/0102198 A1 | 5/2007  | Oxford et al.      | Reed, "Chapter 13: Particle Packing Characteristics," Principles of Ceramics Processing, Second Edition, John Wiley & Sons, Inc., pp. 215-227, 1995.                                                                                                |
| 2007/0102199 A1 | 5/2007  | Smith et al.       | U.S. Appl. No. 60/566,063, filed Apr. 28, 2004, entitled "Body Materials for Earth Boring Bits" to Mirchandani et al.                                                                                                                               |
| 2007/0102200 A1 | 5/2007  | Choe et al.        | Warrier et al., "Infiltration of Titanium Alloy-Matrix Composites," Journal of Materials Science Letters, 12, pp. 865-868, Chapman & Hall, 1993.                                                                                                    |
| 2007/0102202 A1 | 5/2007  | Choe et al.        | Yang, Guang, et al., "Chemical Reaction in Al Matrix Composite Reinforced with SiCp Coated by SnO <sub>2</sub> ," Journal of Materials Science, vol. 39, pp. 3689-3694, 2004.                                                                       |
| 2008/0202814 A1 | 8/2008  | Lyons et al.       | Yuan, R., et al., "Ambient to High-Temperature Fracture Toughness and Cyclic Fatigue Behavior in Al-Containing Silicon Carbide Ceramics," Acta mater., vol. 51, pp. 6477-6491, 2003.                                                                |
| 2009/0031863 A1 | 2/2009  | Lyons et al.       | Zhang, Xiao Feng, et al., "Abrasive Wear Behavior of Heat-Treated ABC-Silicon Carbide," J. Am. Ceram. Soc., vol. 86, No. 8, pp. 1370-1378, 2003.                                                                                                    |
| 2009/0044663 A1 | 2/2009  | Stevens et al.     | US 4,966,627, 10/1990, Keshavan et al. (withdrawn)                                                                                                                                                                                                  |

## FOREIGN PATENT DOCUMENTS

|    |               |         |
|----|---------------|---------|
| CA | 2212197       | 10/2000 |
| EP | 0264674 A2    | 4/1988  |
| EP | 0453428 A1    | 10/1991 |
| EP | 0995876 A2    | 4/2000  |
| EP | 1244531 B1    | 10/2002 |
| GB | 945227        | 12/1963 |
| GB | 2017153       | 10/1979 |
| GB | 2203774 A     | 10/1988 |
| GB | 2345930 A     | 7/2000  |
| GB | 2385350 A     | 8/2003  |
| GB | 2393449 A     | 3/2004  |
| JP | 10219385 A    | 8/1998  |
| WO | 03049889 A2   | 6/2003  |
| WO | 2004053197 A2 | 6/2004  |

## OTHER PUBLICATIONS

- Basavarajappa, S., et al., "Dry Sliding Wear Behaviour of Al 2219/SiC Metal Matrix Composites," Materials Science-Poland, vol. 24, No. 2/1, 2006.
- Chen, D., et al., "High-Temperature Cyclic Fatigue-Crack Growth Behavior in an In Situ Toughened Silicon Carbide," Acta mater., vol. 48, pp. 659-674, 2000.
- Chen, D., et al., "Mechanisms of High-Temperature Fatigue in Silicon Carbide Ceramics," Fatigue and Fracture Behavior of High Temperature Materials, TMS (The Minerals, Metals & Materials Society), Warrendale, PA, pp. 1-8, 2000.
- Chen, D., et al., "Role of the Grain-Boundary Phase on the Elevated-Temperature Strength, Toughness, Fatigue and Creep Resistance of Silicon Carbide Sintered with Al, B and C," Acta mater., vol. 48, pp. 4599-4608, 2000.
- Choe et al., "Effect of Tungsten Additions on the Mechanical Properties of Ti-6Al-4V," Material Science and Engineering, A 396, pp. 99-106, 2005.
- Diamond Innovations, "Composite Diamond Coatings, Superhard Protection of Wear Parts New Coating and Service Parts from Diamond Innovations" Brochure, 7 pages, 2004.
- Gale et al., Smithells Metals Reference Book, Eighth Edition, p. 2117, 2003.
- International Search Report and Written Opinion of the International Search Authority for International Application No. PCT/US2006/043669, mailed Apr. 13, 2007.
- International Search Report and Written Opinion of the International Search Authority for International Application No. PCT/US2006/043670, mailed Apr. 2, 2007.
- International Search Report for International Application No. PCT/US2009/046812 dated Jan. 26, 2010, 5 pages.
- International Search Report for International PCT International Application No. PCT/US2007/023275, mailed Apr. 11, 2008.
- International Written Opinion for International Application No. PCT/US2009/046812 dated Jan. 26, 2010, 5 pages.
- Key-To-Nonferrous, "Aluminum Matrix Composites with Discontinuous Silicon Carbide Reinforcement," <http://www.key-to-nonferrous.com>, 3 pages, downloaded Aug. 27, 2007.
- M Cubed Technologies Inc., "Cast Silicon Carbide Particulate-Reinforced Aluminum (Al/SiC) Metal Matrix Composites," Technote, Cast MMC, Rev. 02, 3 pages, May 8, 2001.
- Mabuchi, M., et al., "Very High Strain-Rate Superplasticity in a Particulate Si<sub>3</sub>N<sub>4</sub>/6061 Aluminum Composite," Scripta Metallurgica et Materialia, vol. 25, No. 11, pp. 2517-2520, Copyright (c) Pergamon Press plc., 1991.
- Miserez et al. "Particle Reinforced Metals of High Ceramic Content," Material Science and Engineering A 387-389, pp. 822-831, Elsevier., 2004.
- Moberlychan, W.J., et al., "Controlling Interface Chemistry and Structure to Process and Toughen Silicon Carbide," Acta mater., vol. 46, No. 7, pp. 2471-2477, 1998.
- Moberlychan, W.J., et al., "The Roles of Amorphous Grain Boundaries and the  $\beta$ - $\alpha$  Transformation in Toughening SiC," Acta mater., vol. 46, No. 5, pp. 1625-1635, 1998.
- PCT International Search Report for International Application No. PCT/US2008/087647, mailed Jul. 23, 2009, 5 pages.
- PCT International Written Opinion for International Application No. PCT/US2008/087647, mailed Jul. 23, 2009, 5 pages.
- Pruthviraj, R.D., et al., "Friction and Wear of Al6061 Containing 10wt.% SiC Metal Matrix Composites," International Journal of Material Science, vol. 2, No. 1, pp. 59-64, 2007.
- Reed, "Chapter 13: Particle Packing Characteristics," Principles of Ceramics Processing, Second Edition, John Wiley & Sons, Inc., pp. 215-227, 1995.
- U.S. Appl. No. 60/566,063, filed Apr. 28, 2004, entitled "Body Materials for Earth Boring Bits" to Mirchandani et al.
- Warrier et al., "Infiltration of Titanium Alloy-Matrix Composites," Journal of Materials Science Letters, 12, pp. 865-868, Chapman & Hall, 1993.
- Yang, Guang, et al., "Chemical Reaction in Al Matrix Composite Reinforced with SiCp Coated by SnO<sub>2</sub>," Journal of Materials Science, vol. 39, pp. 3689-3694, 2004.
- Yuan, R., et al., "Ambient to High-Temperature Fracture Toughness and Cyclic Fatigue Behavior in Al-Containing Silicon Carbide Ceramics," Acta mater., vol. 51, pp. 6477-6491, 2003.
- Zhang, Xiao Feng, et al., "Abrasive Wear Behavior of Heat-Treated ABC-Silicon Carbide," J. Am. Ceram. Soc., vol. 86, No. 8, pp. 1370-1378, 2003.

\* cited by examiner



FIG. 1



FIG. 2



FIG. 3

**FIG. 4**

## 1

**EARTH-BORING TOOLS COMPRISING  
SILICON CARBIDE COMPOSITE  
MATERIALS, AND METHODS OF FORMING  
SAME**

**CROSS-REFERENCE TO RELATED  
APPLICATIONS**

This application is a divisional of U.S. patent application Ser. No. 11/965,018, filed Dec. 27, 2007, now U.S. Pat. No. 7,807,099, issued Oct. 5, 2010, which is a continuation-in-part of U.S. patent application Ser. No. 11/271,153, filed Nov. 10, 2005, now U.S. Pat. No. 7,802,495, issued Sep. 28, 2010, and U.S. patent application Ser. No. 11/272,439, filed Nov. 10, 2005, now U.S. Pat. No. 7,776,256, issued Aug. 17, 2010, the disclosure of each of which is hereby incorporated herein by this reference in its entirety.

**TECHNICAL FIELD**

The present invention generally relates to earth-boring tools, and to methods of manufacturing such earth-boring tools. More particularly, the present invention generally relates to earth-boring tools that include a body having at least a portion thereof substantially formed of a particle-matrix composite material, and to methods of manufacturing such earth-boring tools.

**BACKGROUND**

Rotary drill bits are commonly used for drilling bore holes, or well bores, in earth formations. Rotary drill bits include two primary configurations. One configuration is the roller cone bit, which conventionally includes three roller cones mounted on support legs that extend from a bit body. Each roller cone is configured to spin or rotate on a support leg. Teeth are provided on the outer surfaces of each roller cone for cutting rock and other earth formations. The teeth often are coated with an abrasive, hard (hardfacing) material. Such materials often include tungsten carbide particles dispersed throughout a metal alloy matrix material. Alternatively, receptacles are provided on the outer surfaces of each roller cone into which hard metal inserts are secured to form the cutting elements. In some instances, these inserts comprise a superabrasive material formed on and bonded to a metallic substrate. The roller cone drill bit may be placed in a bore hole such that the roller cones abut against the earth formation to be drilled. As the drill bit is rotated under applied weight on bit, the roller cones roll across the surface of the formation, and the teeth crush the underlying formation.

A second primary configuration of a rotary drill bit is the fixed-cutter bit (often referred to as a "drag" bit), which conventionally includes a plurality of cutting elements secured to a face region of a bit body. Generally, the cutting elements of a fixed-cutter type drill bit have either a disk shape or a substantially cylindrical shape. A hard, superabrasive material, such as mutually bonded particles of polycrystalline diamond, may be provided on a substantially circular end surface of each cutting element to provide a cutting surface. Such cutting elements are often referred to as "polycrystalline diamond compact" (PDC) cutters. The cutting elements may be fabricated separately from the bit body and are secured within pockets formed in the outer surface of the bit body. A bonding material such as an adhesive or a braze alloy may be used to secure the cutting elements to the bit body. The fixed-cutter drill bit may be placed in a bore hole such that the cutting elements abut against the earth formation

## 2

to be drilled. As the drill bit is rotated, the cutting elements scrape across and shear away the surface of the underlying formation.

The bit body of a rotary drill bit of either primary configuration may be secured, as is conventional, to a hardened steel shank having an American Petroleum Institute (API) threaded pin for attaching the drill bit to a drill string. The drill string includes tubular pipe and equipment segments coupled end-to-end between the drill bit and other drilling equipment at the surface. Equipment such as a rotary table or top drive may be used for rotating the drill string and the drill bit within the bore hole. Alternatively, the shank of the drill bit may be coupled directly to the drive shaft of a down-hole motor, which then may be used to rotate the drill bit.

The bit body of a rotary drill bit may be formed from steel. Alternatively, the bit body may be formed from a particle-matrix composite material. Such particle-matrix composite materials conventionally include hard tungsten carbide particles randomly dispersed throughout a copper or copper-based alloy matrix material (often referred to as a "binder" material). Such bit bodies conventionally are formed by embedding a steel blank in tungsten carbide particulate material within a mold, and infiltrating the particulate tungsten carbide material with molten copper or copper-based alloy material. Drill bits that have bit bodies formed from such particle-matrix composite materials may exhibit increased erosion and wear resistance, but lower strength and toughness, relative to drill bits having steel bit bodies.

As subterranean drilling conditions and requirements become ever more rigorous, there arises a need in the art for novel particle-matrix composite materials for use in bit bodies of rotary drill bits that exhibit enhanced physical properties and that may be used to improve the performance of earth-boring rotary drill bits.

**BRIEF SUMMARY OF THE INVENTION**

In some embodiments, the present invention includes earth-boring tools for drilling subterranean formations. The tools include a bit body comprising a composite material. The composite material includes a first discontinuous phase within a continuous matrix phase. The first discontinuous phase includes silicon carbide. In some embodiments, the discontinuous phase may comprise silicon carbide particles, and the continuous matrix phase may comprise aluminum or an aluminum-based alloy. Furthermore, the first discontinuous phase may optionally comprise what may be referred to as an ABC-SiC material, as discussed in further detail below. Optionally, such ABC-SiC materials may comprise toughened ABC-SiC materials that exhibit increased fracture toughness relative to conventional silicon carbide materials.

In further embodiments, the present invention includes methods of forming earth-boring tools. The methods include providing a plurality of silicon carbide particles in a matrix material to form a body, and shaping the body to form at least a portion of an earth-boring tool for drilling subterranean formations. In some embodiments, the silicon carbide particles may comprise an ABC-SiC material. Optionally, such ABC-SiC materials may be toughened to cause the ABC-SiC materials to exhibit increased fracture toughness relative to conventional silicon carbide materials. In some embodiments, silicon carbide particles may be infiltrated with a molten matrix material, such as, for example, an aluminum or aluminum-based alloy. In additional embodiments, a green powder component may be provided that includes a plurality of particles comprising silicon carbide and a plurality of

particles comprising matrix material, and the green powder component may be at least partially sintered.

In still further embodiments, the present invention includes methods of forming at least a portion of an earth-boring tool. An ABC-SiC material may be consolidated to form one or more compacts, and the compacts may be broken apart to form a plurality of ABC-SiC particles. At least a portion of a body of an earth-boring tool may be formed to comprise a composite material that includes the plurality of ABC-SiC particles. Optionally, such ABC-SiC materials may be toughened to cause the ABC-SiC materials to exhibit increased fracture toughness relative to conventional silicon carbide materials.

#### BRIEF DESCRIPTION OF THE SEVERAL VIEWS OF THE DRAWINGS

While the specification concludes with claims particularly pointing out and distinctly claiming that which is regarded as the present invention, the advantages of this invention may be more readily ascertained from the following description of the invention when read in conjunction with the accompanying drawings in which:

FIG. 1 is a partial cross-sectional side view of an earth-boring rotary drill bit that embodies teachings of the present invention and includes a bit body comprising a particle-matrix composite material;

FIG. 2 is an illustration representing one example of how a microstructure of the particle-matrix composite material of the bit body of the drill bit shown in FIG. 1 may appear in a micrograph at a first level of magnification;

FIG. 3 is an illustration representing one example of how the microstructure of the particles of the particle-matrix composite material shown in FIG. 2 may appear at a relatively higher level of magnification; and

FIG. 4 is an illustration representing one example of how the microstructure of the matrix material of the particle-matrix composite material shown in FIG. 2 may appear at a relatively higher level of magnification.

#### DETAILED DESCRIPTION OF THE INVENTION

The illustrations presented herein are not meant to be actual views of any particular material, apparatus, or method, but are merely idealized representations which are employed to describe embodiments of the present invention. Additionally, elements common between figures may retain the same numerical designation.

An embodiment of an earth-boring rotary drill bit 10 of the present invention is shown in FIG. 1. The drill bit 10 includes a bit body 12 comprising a particle-matrix composite material 15 that includes a plurality of silicon carbide particles dispersed throughout an aluminum or an aluminum-based alloy matrix material. By way of example and not limitation, the bit body 12 may include a crown region 14 and a metal blank 16. The crown region 14 may be predominantly comprised of the particle-matrix composite material 15, as shown in FIG. 1. The metal blank 16 may comprise a metal or metal alloy, and may be configured for securing the crown region 14 of the bit body 12 to a metal shank 20 that is configured for securing the drill bit 10 to a drill string (not shown). The metal blank 16 may be secured to the crown region 14 during fabrication of the crown region 14, as discussed in further detail below. In additional embodiments, however, the drill bit 10 may not include a metal blank 16.

FIG. 2 is an illustration providing one example of how the microstructure of the particle-matrix composite material 15

may appear in a magnified micrograph acquired using, for example, an optical microscope, a scanning electron microscope (SEM), or other instrument capable of acquiring or generating a magnified image of the particle-matrix composite material 15. As shown in FIG. 2, the particle-matrix composite material 15 may include a plurality of silicon carbide (SiC) particles 50 dispersed throughout an aluminum or an aluminum-based alloy matrix material 52. In other words, the particle-matrix composite material 15 may include a plurality of discontinuous silicon carbide (SiC) phase regions dispersed throughout a continuous aluminum or an aluminum-based alloy phase. By way of example and not limitation, in some embodiments, the silicon carbide particles 50 may comprise between about forty percent (40%) and about seventy percent (70%) by weight of the particle-matrix composite material 15, and the matrix material 52 may comprise between about thirty percent (30%) and about sixty percent (60%) by weight of the particle-matrix composite material 15. In additional embodiments, the silicon carbide particles 50 may comprise between about seventy percent (70%) and about ninety-five percent (95%) by weight of the particle-matrix composite material 15, and the matrix material 52 may comprise between about thirty percent (30%) and about five percent (5%) by weight of the particle-matrix composite material 15.

As shown in FIG. 2, in some embodiments, the silicon carbide particles 50 may have different sizes. For example, the plurality of silicon carbide particles 50 may include a multi-modal particle size distribution (e.g., bi-modal, tri-modal, tetra-modal, penta-modal, etc.). In other embodiments, however, the silicon carbide particles 50 may have a substantially uniform particle size, which may exhibit a Gaussian or log-normal distribution. By way of example and not limitation, the plurality of silicon carbide particles 50 may include a plurality of -70 ASTM (American Society for Testing and Materials) mesh silicon carbide particles. As used herein, the phrase “-70 ASTM mesh particles” means particles that pass through an ASTM No. 70 U.S.A. standard testing sieve as defined in ASTM Specification E11-04, which is entitled Standard Specification for Wire Cloth and Sieves for Testing Purposes.

The silicon carbide particles 50 may comprise, for example, generally rough, non-rounded (e.g., polyhedron-shaped) particles or generally smooth, rounded particles. In some embodiments, each silicon carbide particle 50 may comprise a plurality of individual silicon carbide grains, which may be bonded to one another. Such interbonded silicon carbide grains in the silicon carbide particles 50 may be generally plate-like, or they may be generally elongated. For example, the interbonded silicon carbide grains may have an aspect ratio (the ratio of the average particle length to the average particle width) of greater than about five (5) (e.g., between about five (5) and about nine (9)).

FIG. 3 illustrates one example of how the microstructure of the silicon carbide particles 50 shown in FIG. 2 may appear at a relatively higher level of magnification. As shown in FIG. 3, each silicon carbide particle 50 may, in some embodiments, comprise a plurality of interlocked elongated and/or plate-shaped grains 51 comprising silicon carbide (and, optionally, an ABC-SiC material, which may comprise an in situ toughened ABC-SiC material).

In some embodiments, the silicon carbide particles 50 may comprise small amounts of aluminum (Al), boron (B), and carbon (C). For example, the silicon carbide material in the silicon carbide particles 50 may comprise between about one percent by weight (1.0 wt %) and about five percent by weight (5.0 wt %) aluminum, less than about one percent by weight (1.0 wt %) boron, and between about one percent by weight

(1.0 wt %) and about four percent by weight (4.0 wt %) carbon. Such silicon carbide materials are referred to in the art as “ABC-SiC” materials, and may exhibit physical properties that are relatively more desirable than conventional SiC materials for purposes of forming the particle-matrix composite material 15 of the bit body 12 of the earth-boring rotary drill bit 10. As one non-limiting example, the silicon carbide material in the silicon carbide particles 50 may comprise about

nese, scandium, silicon, zirconium, and zinc. Furthermore, trace amounts of at least one of silver, gold, and indium optionally may be included in the matrix material 52 to enhance the wettability of the matrix material relative to the silicon carbide particles 50. Table 1 below sets forth various examples of compositions of matrix material 52 that may be used as the particle-matrix composite material 15 of the crown region 14 of the bit body 12 shown in FIG. 1.

TABLE 1

| Example No. | Approximate Elemental Weight Percent |      |      |      |      |      |      |     |      |      |      |      |
|-------------|--------------------------------------|------|------|------|------|------|------|-----|------|------|------|------|
|             | Al                                   | Cu   | Mg   | Mn   | Si   | Zr   | Fe   | Cr  | Ni   | Sn   | Ti   | Zn   |
| 1           | 95.0                                 | 5.0  | —    | —    | —    | —    | —    | —   | —    | —    | —    | —    |
| 2           | 96.5                                 | 3.5  | —    | —    | —    | —    | —    | —   | —    | —    | —    | —    |
| 3           | 94.5                                 | 4.0  | 1.5  | —    | —    | —    | —    | —   | —    | —    | —    | —    |
| 4           | 93.5                                 | 4.4  | 0.5  | 0.8  | 0.8  | —    | —    | —   | —    | —    | —    | —    |
| 5           | 93.4                                 | 4.5  | 1.5  | 0.6  | —    | —    | —    | —   | —    | —    | —    | —    |
| 6           | 93.5                                 | 4.4  | 1.5  | 0.6  | —    | —    | —    | —   | —    | —    | —    | —    |
| 7           | 89.1                                 | 2.3  | 2.3  | —    | —    | 0.1  | —    | —   | —    | —    | —    | 6.2  |
| 8           | 50.0                                 | —    | —    | —    | 50.0 | —    | —    | —   | —    | —    | —    | —    |
| 9           | 99.0                                 | 0.10 | —    | —    | 0.15 | —    | 0.7  | —   | —    | —    | —    | 0.05 |
| 10          | 92.2                                 | 4.5  | 0.30 | 2.5  | 0.10 | —    | 0.15 | —   | —    | —    | 0.25 | —    |
| 11          | 87.3                                 | 3.5  | 0.1  | 0.5  | 6.0  | —    | 1.0  | —   | 0.35 | —    | 0.25 | 1.0  |
| 12          | 83.4                                 | 1.0  | 0.1  | 0.35 | 12.0 | —    | 2.0  | —   | 0.5  | 0.15 | —    | 0.5  |
| 13          | 94.0                                 | 0.15 | 4.25 | 0.35 | 0.35 | 0.15 | 0.5  | —   | —    | —    | 0.25 | —    |
| 14          | 93.5                                 | 0.2  | 1.4  | 0.4  | 0.2  | —    | 0.8  | 0.3 | —    | —    | 0.25 | 2.95 |
| 15          | 90.2                                 | 1.0  | 0.1  | 0.1  | 0.7  | —    | 0.7  | —   | 1.0  | 6.0  | 0.2  | —    |

three percent by weight (3.0 wt %) aluminum, about six tenths of one percent by weight (0.6 wt %) boron, and about two percent by weight (2.0 wt %) carbon. In some embodiments, the silicon carbide particles 50 may comprise an ABC-SiC material that exhibits a fracture toughness of about five megapascals root meters ( $5.0 \text{ MPa}\cdot\text{m}^{1/2}$ ) or more. More particularly, the silicon carbide particles 50 may comprise an ABC-SiC material that exhibits a fracture toughness of about six megapascals root meters ( $6.0 \text{ MPa}\cdot\text{m}^{1/2}$ ) or more. In yet further embodiments, the silicon carbide particles 50 may comprise an ABC-SiC material that exhibits a fracture toughness of about nine megapascals root meters ( $9.0 \text{ MPa}\cdot\text{m}^{1/2}$ ) or more. Optionally, the silicon carbide particles 50 may comprise an in situ toughened ABC-SiC material, as discussed in further detail below. Such in situ toughened ABC-SiC materials may exhibit a fracture toughness greater than about five megapascals root meters ( $5 \text{ MPa}\cdot\text{m}^{1/2}$ ), or even greater than about six megapascals root meters ( $6 \text{ MPa}\cdot\text{m}^{1/2}$ ). In some embodiments, the in situ toughened ABC-SiC materials may exhibit a fracture toughness greater than about nine megapascals root meters ( $9 \text{ MPa}\cdot\text{m}^{1/2}$ ).

In some embodiments, the silicon carbide particles 50 may comprise a coating comprising a material configured to enhance the wettability of the silicon carbide particles 50 to the matrix material 52 and/or to prevent any detrimental chemical reaction from occurring between the silicon carbide particles 50 and the surrounding matrix material 52. By way of example and not limitation, the silicon carbide particles 50 may comprise a coating of at least one of tin oxide ( $\text{SnO}_2$ ), tungsten, nickel, and titanium.

In some embodiments of the present invention, the bulk matrix material 52 may include at least seventy-five percent by weight (75 wt %) aluminum, and at least trace amounts of at least one of boron, carbon, copper, iron, lithium, magnesium, manganese, nickel, scandium, silicon, tin, zirconium, and zinc. Furthermore, in some embodiments, the matrix material 52 may include at least ninety percent by weight (90 wt %) aluminum, and at least three percent by weight (3 wt %) of at least one of boron, carbon, copper, magnesium, manga-

FIG. 4 is an enlarged view of a region of the matrix material 30 52 shown in FIG. 2. FIG. 4 illustrates one example of how the 35 microstructure of the matrix material 52 of the particle-matrix composite material 15 may appear in a micrograph at an even greater magnification level than that represented in FIG. 2. Such a micrograph may be acquired using, for example, a scanning electron microscope (SEM) or a transmission electron 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 833

may impart one or more desirable properties to the matrix material 52, such as, for example, increased hardness. Furthermore, in some embodiments, metastable transition phases may impart one or more physical properties to the matrix material 52 that are more desirable than those imparted to the matrix material 52 by equilibrium precipitate phases (e.g., CuAl<sub>2</sub>).

With continued reference to FIG. 4, the matrix material 52 may include a plurality of grains 60 that abut one another along grain boundaries 62. As shown in FIG. 4, a relatively high concentration of a discontinuous precipitate phase 56 may be present along the grain boundaries 62. In some embodiments of the present invention, the grains 60 of matrix material 52 may have at least one of a size and shape that is tailored to enhance one or more mechanical properties of the matrix material 52. For example, in some embodiments, the grains 60 of matrix material 52 may have a relatively smaller size (e.g., an average grain size of about six microns (6  $\mu\text{m}$ ) or less) to impart increased hardness to the matrix material 52, while in other embodiments, the grains 60 of matrix material 52 may have a relatively larger size (e.g., an average grain size of greater than six microns (6  $\mu\text{m}$ )) to impart increased toughness to the matrix material 52. The size and shape of the grains 60 may be selectively tailored using heat treatments such as, for example, quenching and annealing, as known in the art. Furthermore, at least trace amounts of at least one of titanium and boron optionally may be included in the matrix material 52 to facilitate grain size refinement.

Referring again to FIG. 1, the bit body 12 may be secured to the metal shank 20 by way of, for example, a threaded connection 22 and a weld 24 that extends around the drill bit 10 on an exterior surface thereof along an interface between the bit body 12 and the metal shank 20. The metal shank 20 may be formed from steel, and may include a threaded pin 28 conforming to American Petroleum Institute (API) standards for attaching the drill bit 10 to a drill string (not shown).

As shown in FIG. 1, the bit body 12 may include wings or blades 30 that are separated from one another by junk slots 32. Internal fluid passageways 42 may extend between the face 18 of the bit body 12 and a longitudinal bore 40, which extends through the steel shank 20 and at least partially through the bit body 12. In some embodiments, nozzle inserts (not shown) may be provided at the face 18 of the bit body 12 within the internal fluid passageways 42.

The drill bit 10 may include a plurality of cutting structures on the face 18 thereof. By way of example and not limitation, a plurality of polycrystalline diamond compact (PDC) cutters 34 may be provided on each of the blades 30, as shown in FIG. 1. The PDC cutters 34 may be provided along the blades 30 within pockets 36 formed in the face 18 of the bit body 12, and may be supported from behind by buttresses 38, which may be integrally formed with the crown region 14 of the bit body 12.

The steel blank 16 shown in FIG. 1 may be generally cylindrically tubular. In additional embodiments, the steel blank 16 may have a fairly complex configuration and may include external protrusions corresponding to blades 30 or other features extending on the face 18 of the bit body 12.

The rotary drill bit 10 shown in FIG. 1 may be fabricated by separately forming the bit body 12 and the shank 20, and then attaching the shank 20 and the bit body 12 together. The bit body 12 may be formed by a variety of techniques, some of which are described in further detail below.

In some embodiments, the bit body 12 may be formed using so-called "suspension" or "dispersion" casting techniques. For example, a mold (not shown) may be provided that includes a mold cavity having a size and shape corre-

sponding to the size and shape of the bit body 12. The mold may be formed from, for example, graphite or any other high-temperature refractory material, such as a ceramic. The mold cavity of the mold may be machined using a five-axis machine tool. Fine features may be added to the cavity of the mold using hand-held tools. Additional clay work also may be required to obtain the desired configuration of some features of the bit body 12. Where necessary, preform elements or displacements (which may comprise ceramic components, graphite components, or resin-coated sand compact components) may be positioned within the mold cavity and used to define the internal passageways 42, cutting element pockets 36, junk slots 32, and other external topographic features of the bit body 12.

After forming the mold, a suspension may be prepared that includes a plurality of silicon carbide particles 50 (FIG. 2) suspended within molten matrix material 52. Molten matrix material 52 having a composition as previously described herein then may be prepared by mixing stock material, particulate material, and/or powder material of each of the various elemental constituents in their respective weight percentages in a container and heating the mixture to a temperature sufficient to cause the mixture to melt, forming a molten matrix material 52 of desired composition. After forming the molten matrix material 52 of desired composition, silicon carbide particles 50 may be suspended and dispersed throughout the molten matrix material 52 to form the suspension. As previously mentioned, in some embodiments, the silicon carbide particles 50 may be coated with a material configured to enhance the wettability of the silicon carbide particles 50 to the molten matrix material 52 and/or to prevent any detrimental chemical reaction from occurring between the silicon carbide particles 50 and the molten matrix material 52. By way of example and not limitation, the silicon carbide particles 50 may comprise a coating of tin oxide (SnO<sub>2</sub>).

Optionally, a metal blank 16 (FIG. 1) may be at least partially positioned within the mold such that the suspension may be cast around the metal blank 16 within the mold.

The suspension comprising the silicon carbide particles 50 and molten matrix material 52 may be poured into the mold cavity of the mold. As the molten matrix material 52 (e.g., molten aluminum or aluminum-based alloy materials) may be susceptible to oxidation, the infiltration process may be carried out under vacuum. In additional embodiments, the molten matrix material 52 may be substantially flooded with an inert gas or a reductant gas to prevent oxidation of the molten matrix material 52. In some embodiments, pressure may be applied to the suspension during casting to facilitate the casting process and to substantially prevent the formation of voids within the bit body 12 being formed.

After casting the suspension within the mold, the molten matrix material 52 may be allowed to cool and solidify, forming a solid matrix material 52 of the particle-matrix composite material 15 around the silicon carbide particles 50.

In some embodiments, the bit body 12 may be formed using so-called "infiltration" casting techniques. For example, a mold (not shown) may be provided that includes a mold cavity having a size and shape corresponding to the size and shape of the bit body 12. The mold may be formed from, for example, graphite or any other high-temperature refractory material, such as a ceramic. The mold cavity of the mold may be machined using a five-axis machine tool. Fine features may be added to the cavity of the mold using hand-held tools. Additional clay work also may be required to obtain the desired configuration of some features of the bit body 12. Where necessary, preform elements or displacements (which may comprise ceramic components, graphite components, or

resin-coated sand compact components) may be positioned within the mold cavity and used to define the internal passageways 42, cutting element pockets 36, junk slots 32, and other external topographic features of the bit body 12.

After forming the mold, a plurality of silicon carbide particles 50 (FIG. 2) may be provided within the mold cavity to form a body having a shape that corresponds to at least the crown region 14 of the bit body 12. Optionally, a metal blank 16 (FIG. 1) may be at least partially embedded within the silicon carbide particles 50 such that at least one surface of the blank 16 is exposed to allow subsequent machining of the surface of the metal blank 16 (if necessary) and subsequent attachment to the shank 20.

Molten matrix material 52 having a composition as previously described herein, then may be prepared by mixing stock material, particulate material, and/or powder material of each of the various elemental constituents in their respective weight percentages, heating the mixture to a temperature sufficient to cause the mixture to melt, thereby forming a molten matrix material 52 of desired composition. The molten matrix material 52 then may be allowed or caused to infiltrate the spaces between the silicon carbide particles 50 within the mold cavity. Optionally, pressure may be applied to the molten matrix material 52 to facilitate the infiltration process as necessary or desired. As the molten materials (e.g., molten aluminum or aluminum-based alloy materials) may be susceptible to oxidation, the infiltration process may be carried out under vacuum. In additional embodiments, the molten materials may be substantially flooded with an inert gas or a reductant gas to prevent oxidation of the molten materials. In some embodiments, pressure may be applied to the molten matrix material 52 and silicon carbide particles 50 to facilitate the infiltration process and to substantially prevent the formation of voids within the bit body 12 being formed.

After the silicon carbide particles 50 have been infiltrated with the molten matrix material 52, the molten matrix material 52 may be allowed to cool and solidify, forming the solid matrix material 52 of the particle-matrix composite material 15.

In additional embodiments, reactive infiltration casting techniques may be used to form the bit body 12. By way of example and not limitation, the mass to be infiltrated may comprise carbon, and molten silicon may be added to the molten matrix material 52. The molten silicon may react with the carbon to form silicon carbide as the molten mixture infiltrates the carbon material. In this manner, a reaction may be used to form silicon carbide particles 50 in situ during the infiltration casting process.

In some embodiments, the bit body 12 may be formed using so-called particle compaction and sintering techniques such as, for example, those disclosed in application Ser. No. 11/271,153, filed Nov. 10, 2005, now U.S. Pat. No. 7,802,495, issued Sep. 28, 2010, and application Ser. No. 11/272,439, filed Nov. 10, 2005, now U.S. Pat. No. 7,776,256, issued Aug. 17, 2010. Briefly, a powder mixture may be pressed to form a green bit body or billet, which then may be sintered one or more times to form a bit body 12 having a desired final density.

The powder mixture may include a plurality of silicon carbide particles 50 and a plurality of particles comprising a matrix material 52, as previously described herein. Optionally, the powder mixture may further include additives commonly used when pressing powder mixtures such as, for example, binders for providing lubrication during pressing and for providing structural strength to the pressed powder component, plasticizers for making the binder more pliable,

and lubricants or compaction aids for reducing inter-particle friction. Furthermore, the powder mixture may be milled, which may result in the silicon carbide particles 50 being at least partially coated with matrix material 52.

5 The powder mixture may be pressed (e.g., axially within a mold or die, or substantially isostatically within a mold or container) to form a green bit body. The green bit body may be machined or otherwise shaped to form features such as blades, fluid courses, internal longitudinal bores, cutting element pockets, etc., prior to sintering. In some embodiments, the green bit body (with or without machining) may be partially sintered to form a brown bit body, and the brown bit body may be machined or otherwise shaped to form one or more such features prior to sintering the brown bit body to a desired final density.

10 The sintering processes may include conventional sintering in a vacuum furnace, sintering in a vacuum furnace followed by a conventional hot isostatic pressing process, and sintering immediately followed by isostatic pressing at temperatures near the sintering temperature (often referred to as sinter-HIP). Furthermore, the sintering processes may include subliquidus phase sintering. In other words, the sintering processes may be conducted at temperatures proximate to but below the liquidus line of the phase diagram for the 15 matrix material. For example, the sintering processes described herein may be conducted using a number of different methods known to one of ordinary skill in the art, such as the Rapid Omnidirectional Compaction (ROC) process, the CERACON® process, hot isostatic pressing (HIP), or adaptations of such processes.

20 When the bit body 12 is formed by particle compaction and sintering techniques, the bit body 12 may not include a metal blank 16 and may be secured to the shank 20 by, for example, one or more of brazing, welding, and mechanically interlocking.

25 As previously mentioned, in some embodiments, the silicon carbide particles 50 may comprise an in situ toughened ABC-SiC material. In such embodiments, the bit body 12 may be formed by various methods, including those 30 described below.

35 In some embodiments of methods of forming a bit body 12 of the present invention, particles of ABC-SiC may be consolidated to form relatively larger structures or compacts by, for example, hot pressing particles of ABC-SiC at elevated 40 temperatures (e.g., between about 1,650° C. and about 1,950° C.) and pressures (e.g., about fifty megapascals (50 MPa)) for a period of time (e.g., about one hour) in an inert gas (e.g., argon).

45 After consolidation of the ABC-SiC particles to form relatively larger compacts, the compacts may be annealed to tailor the size and shape of the SiC grains in a manner that enhances the fracture toughness of the ABC-SiC material (e.g., to toughen the ABC-SiC material in situ). By way of example, the relatively larger compacts may be annealed at 50 elevated temperatures (e.g., about 1,000° C. or more) for a time period of about one hour or more) in an inert gas.

55 The consolidated and annealed compacts then may be crushed or otherwise broken up (e.g., in a ball mill or an attritor mill) to form relatively smaller silicon carbide particles 50 comprising the in situ toughened ABC-SiC material. Optionally the relatively smaller silicon carbide particles 50 comprising the in situ toughened ABC-SiC material may be screened to separate the particles into certain particle size ranges, and only selected particle size ranges may be used in 60 forming the bit body 12. The silicon carbide particles 50 comprising the in situ toughened ABC-SiC material then may be used to form the bit body 12 by, for example, using any of

## 11

the suspension casting, infiltration casting, or particle compaction and sintering methods previously described herein.

In additional embodiments of methods of forming a bit body 12 of the present invention, particles of ABC-SiC may be consolidated to form relatively larger compacts as previously described. Prior to annealing (and in situ toughening of the ABC-SiC), however, the relatively larger compacts may be crushed or broken up to form relatively smaller silicon carbide particles 50 comprising the ABC-SiC material. The silicon carbide particles 50 comprising the ABC-SiC material then may be used to form the bit body 12 by, for example, using any of the suspension casting, infiltration casting, or particle compaction and sintering methods previously described herein. A matrix material 52 may be used that has a sufficiently high melting point (e.g., greater than about 1,250° C.) to allow annealing and in situ toughening of the ABC-SiC material after forming the bit body 12 without causing incipient melting of the matrix material 52 or undue dissolution between the matrix material 52 and the silicon carbide particles 50. Such matrix materials 52 may include, for example, cobalt, cobalt-based alloys, nickel, nickel-based alloys, or a combination of such materials. In this manner, the ABC-SiC material may be in situ toughened after forming the bit body 12.

In further embodiments of methods of forming a bit body 12 of the present invention, particles of ABC-SiC may be consolidated to form a first set of relatively larger compacts as previously described. Prior to annealing (and in situ toughening of the ABC-SiC), however, the relatively larger compacts may be crushed or broken up to form relatively smaller silicon carbide particles comprising the ABC-SiC material. A second set of relatively larger compacts may be formed by infiltrating (or otherwise consolidating) the silicon carbide particles 50 comprising the ABC-SiC material with a first material that has a sufficiently high melting point (e.g., greater than about 1,250° C.) to allow annealing and in situ toughening of the ABC-SiC material after infiltrating with the first material. The second set of compacts then may be annealed and in situ toughened, as previously described, after which the second set of compacts may be crushed or otherwise broken up to form the relatively smaller silicon carbide particles 50 comprising in situ toughened ABC-SiC material. The silicon carbide particles 50 comprising the in situ toughened ABC-SiC material then may be used to form the bit body 12 by, for example, using any of the suspension casting, infiltration casting, or particle compaction and sintering methods previously described herein. A matrix material 52 may be used having a melting point such that the bit body 12 may be formed without causing incipient melting of the first material (which is used to infiltrate the ABC-SiC particles prior to in situ toughening), or undue dissolution between the matrix material 52 and the first material or the silicon carbide particles 50.

After or during formation of the bit body 12, the bit body 12 optionally may be subjected to one or more thermal treatments (different than in situ toughening, as previously described) to selectively tailor one or more physical properties of at least one of the matrix material 52 and the silicon carbide particles 50.

For example, the matrix material 52 may be subjected to a precipitation hardening process to form a discontinuous phase 56 comprising precipitates, as previously described in relation to FIG. 4. For example, the matrix material 52 may comprise between about 95% and about 96.5% by weight aluminum and between about 3.5% and about 5% by weight copper, as previously described. In fabricating the bit body 12 in an infiltration casting type process, as described above, the

## 12

matrix material 52 may be heated to a temperature of greater than about 548° C. (a eutectic temperature for the particular alloy) for a sufficient time to allow the composition of the molten matrix material 52 to become substantially homogeneous. The substantially homogenous molten matrix material 52 may be poured into a mold cavity and allowed to infiltrate the spaces between silicon carbide particles 50 within the mold cavity. After substantially complete infiltration of the silicon carbide particles 50, the temperature of the molten matrix material 52 may be cooled relatively rapidly (i.e., quenched) to a temperature of less than about 100° C. to cause the matrix material 52 to solidify without formation of a significant amount of discontinuous precipitate phases. The temperature of the matrix material 52 then may be heated to a temperature of between about 100° C. and about 548° C. for a sufficient amount of time to allow the formation of a selected amount of discontinuous precipitate phase (e.g., metastable transition precipitation phases, and/or equilibrium precipitation phases). In additional embodiments, the composition of the matrix material 52 may be selected to allow a pre-selected amount of precipitation hardening within the matrix material 52 over time and under ambient temperatures and/or temperatures attained while drilling with the drill bit 10, thereby eliminating the need for a heat treatment at elevated temperatures.

Tungsten carbide materials have been used for many years to form bodies of earth-boring tools. Silicon carbide generally exhibits higher hardness than tungsten carbide materials. Silicon carbide materials also may exhibit superior wear resistance and erosion resistance relative to tungsten carbide materials. Therefore, embodiments of the present invention may provide earth-boring tools that exhibit relatively higher hardness, improved wear resistance, and/or improved erosion resistance relative to conventional tools comprising tungsten carbide composite materials. Furthermore, by employing toughened silicon carbide materials, as disclosed herein, earth-boring tools may be provided that comprise silicon carbide composite materials that exhibit increased fracture toughness.

While the present invention is described herein in relation to embodiments of concentric earth-boring rotary drill bits that include fixed cutters and to embodiments of methods for forming such drill bits, the present invention also encompasses other types of earth-boring tools such as, for example, core bits, eccentric bits, bicenter bits, reamers, mills, and roller cone bits, as well as methods for forming such tools. Thus, as employed herein, the term "bit body" includes and encompasses bodies of all of the foregoing structures, as well as components and subcomponents of such structures.

While the present invention has been described herein with respect to certain preferred embodiments, those of ordinary skill in the art will recognize and appreciate that it is not so limited. Rather, many additions, deletions and modifications to the preferred embodiments may be made without departing from the scope of the invention as hereinafter claimed. In addition, features from one embodiment may be combined with features of another embodiment while still being encompassed within the scope of the invention as contemplated by the inventors. Further, the invention has utility in drill bits and core bits having different and various bit profiles as well as cutter types.

What is claimed is:

1. An earth-boring tool for drilling subterranean formations, the tool comprising:  
a bit body including a crown region comprising a particle-matrix composite material, the particle-matrix composite material comprising a plurality of silicon carbide

## 13

particles dispersed throughout an aluminum or an aluminum-based alloy matrix material, the silicon carbide particles of the plurality of silicon carbide particles comprising between about one percent by weight (1 wt %) and about five percent by weight (5 wt %) aluminum, between zero percent by weight (0 wt %) and about one percent by weight (1 wt %) boron, and between about one percent by weight (1 wt %) and about four percent by weight (4 wt %) carbon; and at least one cutting structure disposed on a face of the bit body.

2. The earth-boring tool of claim 1, wherein the plurality of silicon carbide particles comprises between about 40% and about 70% by weight of the particle-matrix composite material, and wherein the aluminum or aluminum-based alloy matrix material comprises between about 30% and about 60% by weight of the particle-matrix composite material.

3. The earth-boring tool of claim 1, wherein the aluminum or aluminum-based alloy matrix material of the particle-matrix composite material comprises at least 75% by weight aluminum and at least trace amounts of at least one of boron, carbon, copper, iron, lithium, magnesium, manganese, nickel, scandium, silicon, tin, zirconium, and zinc.

4. The earth-boring tool of claim 1, wherein the aluminum or aluminum-based alloy matrix material of the particle-matrix composite material comprises at least one discontinuous precipitate phase dispersed through a continuous phase comprising a solid solution.

5. An earth-boring tool for drilling subterranean formations, the tool comprising:

a bit body comprising a composite material, the composite material comprising a first discontinuous phase dispersed throughout a continuous matrix phase, the first discontinuous phase comprising a silicon carbide material including between about one percent by weight (1 wt %) and about five percent by weight (5 wt %) aluminum, between zero percent by weight (0 wt %) and about one percent by weight (1 wt %) boron, and between about one percent by weight (1 wt %) and about four percent by weight (4 wt %) carbon.

6. The earth-boring tool of claim 5, wherein the silicon carbide material comprises a toughened silicon carbide material and exhibits a fracture toughness greater than about 5 MPa·m<sup>1/2</sup>.

## 14

7. The earth-boring tool of claim 5, wherein the matrix phase comprises at least 75% by weight aluminum and at least trace amounts of at least one of boron, carbon, copper, iron, lithium, magnesium, manganese, nickel, scandium, silicon, tin, zirconium, and zinc.

8. A method of forming an earth-boring tool, the method comprising:

providing a plurality of silicon carbide particles within a cavity of a mold, the cavity having a shape corresponding to at least a portion of a bit body of an earth-boring tool for drilling subterranean formations, providing the plurality of silicon carbide particles comprising:

selecting the silicon carbide material to comprise between about one percent by weight (1 wt %) and about five percent by weight (5 wt %) aluminum, between zero percent by weight (0 wt %) and about one percent by weight (1 wt %) boron, and between about one percent by weight (1 wt %) and about four percent by weight (4 wt %) carbon;

infiltrating the plurality of silicon carbide particles with a molten aluminum or aluminum-based material; and cooling the molten aluminum or aluminum-based material to form a solid matrix material surrounding the plurality of silicon carbide particles.

9. The method of claim 8, further comprising heat treating the solid matrix material to increase the hardness of the solid matrix material.

10. The method of claim 8, wherein infiltrating the plurality of silicon carbide particles comprises infiltrating the plurality of silicon carbide particles with a molten material comprising at least 75% by weight aluminum and at least trace amounts of at least one of copper, iron, lithium, magnesium, manganese, nickel, scandium, silicon, tin, zirconium, and zinc.

11. The method of claim 8, further comprising: cooling the molten material to form a solid solution; and forming at least one discontinuous precipitate phase within the solid solution, the at least one discontinuous precipitate phase causing the solid matrix material to exhibit a bulk hardness that is harder than a bulk hardness of the solid solution.

\* \* \* \* \*